

4 Sheets--Sheet 1.

C. TESSIE du MOTAY.  
Process for Treating Copper Ores.

No. 234,212.

Patented Nov. 9, 1880.



Figure 1.

Witnesses:

Geo. W. Micht  
Alfred J.

Inventor:  
Cyprian Tessie du Motay  
By his attorney  
E. W. Dickerson Jr.

4 Sheets—Sheet 2.

C. TESSIE du MOTAY.  
Process for Treating Copper Ores.

No. 234,212.

Patented Nov. 9, 1880.

Figure 2.



Witnesses:

Geo. W. Miat  
A. Grefe

Inventor:

Cyprien Tessie du Motay  
By his Attorney,  
E. N. Dickerson, Jr.

4 Sheets—Sheet 3.

C. TESSIE du MOTAY.  
Process for Treating Copper Ores.

No. 234,212.

Patented Nov. 9, 1880.



4 Sheets—Sheet 4.

C. TESSIE du MOTAY.  
Process for Treating Copper Ores.

No. 234,212.

Patented Nov. 9, 1880.

*Figure 4*



Witnesses:  
Geo. W. Math  
Alfred J.  
*[Signature]*

Inventor:  
Cyprien Tessie du Motay  
By his Attorney  
E. N. Dickerson

# UNITED STATES PATENT OFFICE.

CYPRIEN TESSIÉ DU MOTAY, OF NEW YORK, N. Y., ASSIGNOR TO EDWARD STERN, OF SAME PLACE.

## PROCESS OF TREATING COPPER ORES.

SPECIFICATION forming part of Letters Patent No. 234,212, dated November 9, 1880.

Application filed November 18, 1879.

*To all whom it may concern:*

Be it known that I, CYPRIEN TESSIÉ DU MOTAY, of the city, county, and State of New York, have invented a new and useful Process 5 of Treating Copper Ores, of which the following is a full, true, and exact description, reference being had to the accompanying drawings.

My process is especially applicable to copper pyrites, being the double sulphides of iron and copper. These ores have hitherto been very difficult to reduce, the expense of the process being generally more than the value of the result. My process, however, is very 15 simple and inexpensive, requiring but little fuel, and reducing the pyrites in one operation to the state of metallic copper. The manner of treating the pyrites is by forcing through them, while in a melted condition, air, steam, 20 and a combustible gas, in a manner to be hereinafter explained.

The apparatus used in carrying out my process is plainly shown in the accompanying drawings, in which—

25 Figure 1 represents a vertical section through my reducing-furnace; Fig. 2, a section through Fig. 1 on the line X X; Fig. 3, a section on the line Y Y through Fig. 1. Fig. 4 represents a vertical section of a modified form of 30 my apparatus.

My apparatus consists, generally, in a chamber or furnace so constructed as to contain the melted ores to be treated, and to facilitate the forcing through the ores in a molten condition 35 of the various gases before referred to. In the form shown in Figs. 1, 2, and 3 it consists, generally, of a U-shaped chamber or furnace, one end being closed and the other being open for the escape of the gases, and connected with 40 the chimney G, as shown. The chamber is divided, as shown, by a partition, R, provided with an opening, O, at its bottom. In other words, the divided partition does not entirely separate the chamber.

45 Arranged to communicate with the closed portion of the chamber are three reservoirs, containing the gas, steam, and air to be used, lettered, respectively, A, B, and C. These communicate with the furnaces by pipes a, b,

and c, each provided with a valve, v, as shown. 50 The vessel A contains a combustible gas, preferably that known as "water-gas," at a suitable pressure—say, of three or four atmospheres. The vessel B contains steam, preferably super-heated, and at about the same pressure. The 55 vessel C contains compressed air, also at about the same pressure.

The steam used in the vessel B may be produced by the same apparatus which makes the water-gas contained in the vessel A; or the 60 vessel B may represent a boiler preferably provided with a suitable superheating apparatus. The furnace F is also provided with a suitable supply-aperture, P, and a delivery-aperture, D. These are arranged to be properly closed 65 by plugs or valves, as shown.

The copper pyrites, having been first melted in an apparatus suitably arranged, are caused to flow into the furnace F through the supply-opening P. The vessel containing compressed 70 air, which air may also be heated, is put in communication, by means of the tube C, with the closed portion of the furnace-chamber. The pressure existing in this portion forces the air downward and through the melted 75 pyrites beneath. The result of this operation is, that the sulphur oxidizes, burning with great heat, serving to still further liquefy the mass, and leaves it in the condition of mingled oxide and protoxide of iron and oxide and 80 protoxide of copper. The communication with the reservoir of steam is then opened, which causes the mingled air and steam to pass through the molten mass. The result of this is the conversion of the oxide and protoxide 85 of copper into the protoxide of copper, and the protoxide of copper, being heavier, falls to the bottom and the protoxide of iron floats on its surface. As soon as all the sulphur has been oxidized, which is known by the circumstance 90 that sulphurous acid is no longer formed, the supply of steam is cut off, and the third reservoir, containing the combustible gas, is put in communication with the closed end of the furnace. This gas, mingling with the air which 95 is being supplied through the pipe C, burns with great intensity, and thoroughly liquefies the iron and copper contained in the furnace.

The gas used should be one containing a certain amount of hydrogen, either free or in combination with a gas, and a certain amount of water in the condition of steam. The supplies of air and of combustible gas are so regulated that the resulting flame is a reducing flame, the gas being in excess of the quantity which can be burned with the air. The result of this operation is, that the protoxide of copper is reduced to the condition of metallic copper; but the protoxide of iron is not reduced, owing to the presence of the water of combustion. When this has been thoroughly accomplished, the delivery aperture is opened and the melted copper is allowed to flow out through the aperture D. The melted protoxide of iron follows, and may be received in a separate receptacle, or may be allowed to fall upon the top of the copper, from which, when cool, it is easily separated by a blow.

Fig. 4 represents a modification, in which an annular partition divides a cylindrical retort into two portions, the inner one being closed for the reception of the gas, steam, or air, before referred to, and the outer or annular chamber being in communication with the atmosphere by chimney G. The gas escapes from the inner chamber through the annular cham-

ber O, and so into the atmosphere. The operation is precisely similar.

I do not claim, broadly, the use of steam for the purpose of separating copper from iron, that being old in the art.

What I claim as my invention, and desire to secure by Letters Patent, is—

1. The process of separating the oxides of copper and iron produced from pyrites, which consists in forcing air through them when melted, thereby reducing them to the condition of mingled oxides and protoxides of iron and copper, and subsequently separating the copper from the iron by forcing steam through the melted mass, substantially as described.

2. The process of producing metallic copper from copper pyrites, which consists in forcing air and steam through the molten mass, thereby reducing it to a condition of mingled protoxide of copper and iron, and subsequently treating them with a reducing-flame containing hydrogen and water, thereby reducing the protoxide of copper to metallic copper, substantially as described.

#### C. TESSIÉ DU MOTAY.

Witnesses:

S. F. SULLIVAN,  
Wm. A. POLLOCK.